

## UNITED STATES PATENT OFFICE.

GUILLAUME WEBER, OF HAYANGE, FRANCE, ASSIGNOR TO LES PETITS FILS DE FRANÇOIS DE WENDEL & CIE, OF HAYANGE, MOSELLE, FRANCE.

## EXPLOSIVE USING LIQUID OXYGEN.

No Drawing.

Application filed January 4, 1923. Serial No. 610,703.

*To all whom it may concern:*

Be it known that I, GUILLAUME WEBER, citizen of the French Republic, residing at Hayange, Moselle, in the Republic of France, have invented new and useful Improvements in Explosives Using Liquid Oxygen, of which the following is a specification.

It is already known to use an explosive based upon liquid air, consisting of a cartridge containing a combustible substance, liquid air and a small cartridge or bag filled with aluminium powder and wherein the detonator is also disposed.

The presence of the detonator in the cartridge has great drawbacks. By a shock or by pushing, one can produce the explosion of the detonator even before the impregnation of the cartridge with liquid air. After its saturation with liquid air or oxygen, a shock or a spark may suffice to cause the explosion of the cartridge. Again, the manufacture of such a cartridge is more complex and expensive.

According to the invention; and in order to obviate these drawbacks, one eliminates the detonator from the small cartridge or bag which contains the aluminium powder or any other metal powder or still a mixture of several combustible powders, and after the cartridge has been impregnated with

liquid oxygen and placed into a blast hole or blast chamber in a mine, it is exploded either by the use of an ordinary cord fuse (Bickford cord) or by means of electric ignition. It has in fact been ascertained that cartridges so constructed, when they do not contain hydrocarbons, will deflagrate in the open air by the action of a flame or a spark. If the cartridge contains hydrocarbons in large proportion, it will detonate after having been submitted to fire.

Having now described my invention, what I claim as new and desire to secure by Letters Patent is:

1. An explosive cartridge comprising an envelope, a combustible absorbent substance in said envelope adapted to be impregnated with liquid oxygen, a metallic powder and a small cartridge or bag inside said envelope containing said metallic powder and containing no detonator.

2. An explosive cartridge comprising an envelope combustible absorbent substances in said envelope adapted to be impregnated with liquid oxygen, metallic powders, and a small cartridge or bag inside said envelope containing said metallic powders and containing no detonator.

In testimony whereof I have signed my name to this specification.

GUILLAUME WEBER.